

Patented Feb. 12, 1929.

1,701,868

# UNITED STATES PATENT OFFICE.

STANLEY L. WILLIS AND WATSON H. WOODFORD, OF BRIDGEPORT, CONNECTICUT, AS  
SIGNORS TO REMINGTON ARMS COMPANY, INC., A CORPORATION OF DELAWARE.

## WATERPROOFING.

No Drawing.

Application filed May 12, 1925. Serial No. 29,798.

This invention relates to the manufacture of waterproof loaded shot shells or cartridges and particularly to the waterproofing of the top wad and the provision of a waterproof joint between the top wad and the shell body.

In the manufacture of shot shells or cartridges, paper tubes for the shot shell bodies are rolled on a mandrel from a sheet of paper and secured by a suitable adhesive. The tube thus formed is waterproofed by the application thereto of a suitable waterproofing composition such for example, as the waterproofing composition disclosed in our copending application Ser. No. 29,797, filed May 12, 1925. To one end of the tube thus formed, a metallic head comprising a primer and a base wad is attached and a charge of powder, wadding and shot is then introduced through the open end of the tube. Upon the shot a closing or top wad is placed and the extending end of the shell tube is turned inward and downward or "crimped" against the top wad to securely hold the charge and the top wad in place.

It is of the greatest importance that not only the top wad, but also the periphery and the inturned end of the shell tube, and the joint between the tube and the top wad be resistant to moisture; since the absorption of moisture by the wad or the tube causes these parts to swell and to become soft and flabby, while moisture within the shell deteriorates the powder. It is therefore necessary that the top wad, the crimp and the joint be carefully waterproofed.

The present invention comprises the discovery that a polymerizable oil or a composition including a polymerizable oil as an essential ingredient is a singularly effective agent for waterproofing the top wad and crimp. The waterproofing material may be applied after the top wad is in place, and either before or after the "crimping" operation. While a number of compositions comprising a polymerizable oil as their essential ingredient have been found to be satisfactory for this purpose, a preferred composition consists of a mixture of a polymerizable oil and one of the class of substances known as "driers", the prime function of the drier being to facilitate oxidation. To the mixture of a polymerizable oil with a drier, a suitable volatile solvent may be added for the purpose of facilitating

spreading the oil and insuring that the oil penetrates and waterproofs the joint between the top wad and the shell body. According to a preferred method of preparing the waterproofing composition, the polymerizable oil and the drier in suitable proportions are heated together to a temperature which will vary with the particular oil and the particular drier used. The appropriate quantity of volatile solvent is added to the heated mixture which is allowed to cool. After cooling, a small quantity of the polymerizable oil may be added as it has been found that such an addition serves to retard the drying of the oil and to insure a more perfect waterproofing. One composition which has been found to give very satisfactory results comprises Chinese wood oil and a drier of manganese resinate and lead oxide, digested in carbon tetrachloride, this composition being prepared as follows: A mixture comprising about 37 parts of Chinese wood oil, one part of manganese resinate and eight parts of lead oxide is brought to the temperature of about 220° C. and maintained at this temperature for a period of about ten minutes. Ninety-five parts of carbon tetrachloride are then added and the composition is allowed to cool. After cooling a small quantity of the Chinese wood oil is added. Other driers such as lead tungate, lead resinate, or cobalt tungate may be used, or the drier may be omitted altogether, likewise other volatile solvents, such as gasoline, turpentine and kerosene may be used. For example, excellent results can be obtained by a mixture comprising sixty parts of Chinese wood oil, fifteen parts of gasoline and fifteen parts of carbon tetrachloride. This formula, however, like the formula above mentioned is illustrative rather than restrictive.

After the application of polymerizable oil or the polymerizable oil compound, the oil is gelatinized by any suitable means such as the exposure to heat, chemical agents, gases or air at ordinary temperature. A very satisfactory drying is effected by exposure to the air for periods varying from two to five hours.

We claim:

1. A loaded paper shot cartridge having the top wad and the crimp sealed and impregnated with a composition containing a polymerizable oil and a drier comprising

manganese resinate and lead oxide in suitable proportions.

2. A loaded paper shot cartridge having the top wad and the crimp sealed and impregnated with a composition containing a polymerizable oil and a drier of manganese resinate and lead oxide digested in a suitable volatile solvent.

3. A loaded paper shot cartridge having the top wad and the crimp sealed and impregnated with a composition containing a polymerizable oil and a drier containing manganese resinate and lead oxide in the proportions of one part of manganese resinate to eight parts of lead oxide.

4. A loaded paper shot cartridge having the top wad and the crimp sealed and impregnated with a composition containing Chinese wood oil, manganese resinate, and

lead oxide, and carbon tetrachloride in the following proportions:

|                      | Parts  |
|----------------------|--------|
| Chinese wood oil     | 37.5   |
| Manganese resinate   | 1.     |
| Lead oxide           | 8.     |
| Carbon tetrachloride | 95. 25 |

5. A loaded paper shot cartridge having the top wad and the crimp sealed and impregnated with a composition containing substantially 37.5 parts of Chinese wood oil, 1 part of manganese resinate and 8 parts of lead oxide heated to about 220° C. and digested in 95 parts of carbon tetrachloride, and having a small quantity of Chinese wood oil added thereto, subsequent to cooling.

STANLEY L. WILLIS.  
WATSON H. WOODFORD.